

1

3,316,328

**STEREOREGULAR POLYOLEFIN  
COMPOSITIONS**

Jack J. Press, Teaneck, N.J., assignor to Iowa Manufacturing Company, Cedar Rapids, Iowa  
No Drawing. Filed Nov. 30, 1964, Ser. No. 414,919  
6 Claims. (Cl. 260—895)

This application is a continuation-in-part of my co-pending application Ser. No. 113,972, filed Apr. 4, 1961, now abandoned.

The invention described herein may be manufactured and used by or for the Government of the United States of America for governmental purposes without the payment of any royalties thereon or therefor.

This invention relates to stereoregular polyolefins. More particularly, this invention relates to polymeric compositions having improved affinity for dyes, said compositions containing a major amount of stereoregular polyolefins.

It is known that polyethylene is unsuitable for the production of textile fibers due to the relatively poor properties imparted to the product. For one thing, staple polyethylene fiber will not hold a crimp and this is necessary for textile processing. For another, it is useless to make a textured or stretch yarn from a continuous filament polyethylene yarn because the characteristics imparted to the yarn are not maintained during weaving, dyeing, or ordinary use. Further, the material from which a fabric is made must be thermally stable before it may be subjected to ordinary use. It must not have a relatively low melting point, and the final fabric must not have a high degree of heat sensitivity, nor relatively soft mechanical properties at elevated temperatures. However, the thermal properties of a polyethylene fabric are such that it is impossible to subject it to ordinary ironing without physically damaging the fabric and it has been found to shrink in the conventional dryer. As is apparent from the foregoing, polyethylene cannot be utilized in the manufacture of everyday fabrics for ordinary use.

In recent times, it has been found that certain linear crystalline hydrocarbon polymers containing stereoregular macromolecules and having melting points between 150° and 300° C. can be used for the production of textile fibers without the inherent difficulties encountered with the use of polyethylene polymers for this purpose. Aside from melting point differences, polypropylene with a tertiary carbon and a methyl side chain, crystallizes differently and has a much higher resilience and elasticity. These properties are essential in generally useful textile fiber. Further, polymers of olefinic hydrocarbons containing stereoregular macromolecules, such as polypropylene, polymethylpentene, and polymethylbutene offer considerable advantages in the production of fibers, particularly because of their good mechanical properties and light weight. However, such polymers have not been satisfactory because of their poor affinity for dyes, this poor affinity being due to the particular chemical nature of such polyolefinic hydrocarbons.

Many processes have been proposed in order to improve the affinity of such polyolefinic hydrocarbons for dyes, such as the addition of soluble solid substances to the molten polyolefin before spinning. The addition of basic substances facilitates dyeing with acid dyes, whereas the addition of acid substances favors dyeing with basic dyes. However, such processes have not been completely satisfactory because soluble modifiers interfere with crystallization, impair strength and are not sufficiently available in the amorphous regions where dyeing takes place.

It has also been proposed to increase the affinity for dyes of polyolefin fibers by grafting monomers onto the

2

fibers after subjecting the fibers to a preliminary peroxidation or to high energy radiation. When such processes are applied to the polyolefin, after it is in filamentary form, the surface properties of the grafted fibers are considerably modified and the dye receptivity is improved. However, when such processes are applied to highly crystalline filaments, any grafting onto the preformed fibers takes place only at the surface. Therefore, subsequent dyeing is limited to the surface portion of the fiber and the dye does not penetrate inside the fiber.

In my copending application titled Modification of Stereoregular Polyolefins, Ser. No. 400,611, filed Sept. 30, 1964, I show the use of selected hydrophilic polymers to improve the dyeability of stereoregular, high melting, polyolefins. The level of addition ranges from 2 to 20% by weight based on the polyolefin. However, my hydrophilic, polymeric, modifiers show only limited dyeability with selected small disperse dyes, and only negligible dyeability with larger ionic dyes such as acid, basic, premetallized and direct dyes. The latter dyes are particularly desirable because of their generally better wash, dry clean, and light fastness properties. The depth and range of dyeability can be increased somewhat by increasing either the molecular weight or the level of addition of the primary modifier. However, increasing the molecular weight makes melt dispersion more difficult and increased levels of addition are not economically feasible and adversely affect physical properties, particularly fibrillation.

In another of my copending applications titled "Modification of Stereoregular Polyolefins With Synergistic Combinations," Ser. No. 406,631, filed Oct. 26, 1964, I teach that, even at low levels of addition, I obtain synergistic improvements in dyeability by replacing between 5% and 50% of the above primary hydrophilic modifiers with selected liquid, wax, or polymeric secondary modifiers having negligible dyeability by themselves. These secondary modifiers are generally low molecular weight additives or possess melting points somewhat lower than the polyolefin itself. These secondary additives associate themselves with the primary hydrophilic polymeric modifier in such a way as to give synergistic combinations that are fusible at temperatures not exceeding the temperature of processing of the polyolefin and have improved processability and dyeability.

However, for optimum efficiency, the primary hydrophilic polymer and the secondary additives must be chosen and processed so that, when dispersed in the polyolefin, the primary and secondary additive will interact uniformly and efficiently to give a complex with improved synergistic utility. In actual practice, it is somewhat difficult to achieve and maintain optimum complex formation before and during melt mixing with the polyolefin. In addition, secondary additives which have not complexed with the hydrophilic polymer may sweat out of the polyolefin and interfere with processing.

Now, I have discovered that the affinity of the polyolefins for dyes may be further improved, over and above the improvement achieved with the above polymeric materials, and comparable with the improvement achieved with the above secondary polar additives, if the modifier incorporated in the polyolefin is one of a specified class of copolymers. Thus, the difficulties encountered with the use of secondary additives are eliminated while the improvement achieved is maintained. As an added advantage, the amount of modifier necessary to achieve a given level of dyeability is reduced. Also, the elimination of secondary additives tends towards greater uniformity in dyeing when the polyolefinic combination is processed under high speed commercial operations.

It is therefore an object of this invention to provide a polymeric composition having improved affinity for dyes

void of the difficulties of the prior art heretofore escribed.

This invention relates to stereoregular polyolefins having increased affinity for dyes and other polar substances comprising:

A matrix of a stereoregular polyolefin taken from the group consisting of polypropylene, polymethylpentene, and polymethylbutene, said matrix of polyolefin having dispersed therein between about 2% and 20% of a modifying copolymer derived from the combination of an oxygen containing N-alkenyl heterocyclic monomeric unit with a monomeric unit containing an amino nitrogen, said copolymer selected from the group consisting of:

- (1) 80% N-vinyl pyrrolidone/20% dimethylaminoethyl methacrylate,
  - (2) 95% N-vinyl pyrrolidone/5% trimethylaminoethyl methacrylate,
  - (3) 85% N-vinyl pyrrolidone/15% trimethylaminomethyl styrene,
  - (4) 80% N-vinyl pyrrolidone/20% methyl ethylene imine,
  - (5) 80% N-isoprenyl pyrrolidone/20% diethylaminoethyl acrylate,
  - (6) 70% N-isoprenyl pyrrolidone/30% dimethylaminoethyl acrylamide,
  - (7) 90% N-acrylyl pyrrolidone/10% N-vinyl pyrrole,
  - (8) 90% N-vinyl methylpyrrolidone/10% lauryldimethylaminoethyl methacrylate,
  - (9) 70% N-vinyl morpholine/30% N-vinyl carbazole,
  - (10) 70% N-vinyl morpholinone/30% N-vinyl indole,
  - (11) 70% N-vinyl morpholinone/30% N-butyl vinyl quinoline,
  - (12) 80% N-vinyl caprolactam/20% N-methyl vinyl imidazole,
  - (13) 80% N-vinyl caprolactam/20% N-vinyl succinimide,
  - (14) 95% N-vinyl oxazolidinone/5% laurylaminoethyl methacrylate,
  - (15) 90% N-vinyl morpholinone/10% butyldimethylaminoethyl methacrylate,
  - (16) 70% N-vinyl benzamidazole/30% N-vinyl diphenylamine,
  - (17) 70% N-vinyl phthalamide/30% N-methyl vinyl piperidine,
  - (18) 90% N-vinyl diglycolimide/10% dimethyl 2-vinyl pyridine,
  - (19) 70% N-vinyl methylpyrrolidone/30% butylaminoethyl methacrylate,
  - (20) 90% N-vinyl pyrrolidone/10% 2-vinyl pyridine,
- all said percentages being percent by weight.

My selected copolymer modifiers contain at least 70% of an oxygen containing N-alkenyl heterocyclic monomeric unit in order to obtain good dye penetration without surface blocking, strong dye affinity and good wash, dry clean, and light fastness. Also, my selected copolymeric modifiers, which should have a molecular weight of at least 10,000, and preferably over 20,000, are strongly hydrophilic, generally soluble in water or an oxygenated solvent, fusible, insoluble but dispersible in polyolefin, and possess melting points of at least 50° C. but preferably over 100° C.

The stereoregular polyolefins which may be used within the concept of this invention include isotactic and syndiotactic polyolefins. These materials are usually made by utilizing stereo-specific catalysts which give polymers which are substantially linear and which develop a high degree of crystallinity.

The following examples will illustrate the utility of the present composition.

#### Example 1

Using conventional solution polymerization procedures, a 50% by weight solution in ethyl alcohol of a 80/20 weight ratio of N-vinyl pyrrolidone/dimethylaminoethyl methacrylate copolymer was prepared. The copolymer had a molecular weight of 40,000.

An aliquot of the above solution was poured into a shallow pan and dried in a forced air circulation oven at a temperature of 50° C. The solid polymer sheet was broken up and then ground in a centrifugal grinder to give a powder passing through a 50 mesh screen.

Portions of the copolymers, in solution and ground forms, were combined in several variations with a representative stereoregular polyolefin, processed into fiber and evaluated using the following procedure:

- 10 (a) Fourteen parts of the 50% ethyl alcohol copolymer solution was uniformly mixed in a laboratory mortar with 93 parts of a powdered (50 to 200 mesh) commercial isotactic polypropylene (molecular weight of about 350,000; melting point of about 170° C.; melt flow index of 3.3; and isotacticity of 95%).
- (b) The polypropylene-modifier mixture was air dried overnight and then dried in an oven at 80° C. until all of the solvent had been removed.
- (c) The coated dry powder was then melt mixed in a screw extruder, forced through a die at 260° C., and collected at ambient temperature on a reel as a 30 denier filament. The filament was heat stretched 300% to give a strong, oriented 10 denier fiber and was then wound into skeins for use in evaluating uniformity of dispersion and dyeability.
- (d) The fiber skeins were scoured with detergent at 80° C., dyed at the boil for one hour at a 20 to 1 bath to fiber ratio with representative dye solutions, and then well scoured to remove any surface dye. The dyed fiber was then evaluated for laundering (74° C.), dry cleaning (Stoddard and perchlorethylene solvents), and light fastness using standard procedures.

One to eight percent dyeings, on weight of fiber (o.w.f.) were carried out with the following dyes:

|                          | Percent o.w.f. |
|--------------------------|----------------|
| Disperse dyes:           |                |
| C.I. disperse blue 7     | 2              |
| C.I. disperse violet 8   | 1              |
| C.I. disperse red 13     | 1              |
| Acid dyes:               |                |
| C.I. acid red 115        | 1              |
| C.I. acid blue 7         | 4              |
| Premetallized acid dyes: |                |
| C.I. acid red 182        | 0.5            |
| C.I. acid black 52       | 8              |
| Mordant dyes:            |                |
| C.I. mordant yellow 1    | 1              |
| C.I. mordant orange 1    | 1              |
| Direct dyes:             |                |
| C.I. direct red 75       | 1              |
| C.I. direct blue 82      | 1              |

An overall rating (poor=0, fair=x, good=xx, and excellent=xxx) was assigned for each dyestuff class based on dyestuff exhaustion and build-up, as well as, wash, dry clean and light fastness as follows:

| 60 | Dyestuff Class |      |                    |         |        |
|----|----------------|------|--------------------|---------|--------|
|    | Disperse       | Acid | Premetallized Acid | Mordant | Direct |
|    | Rating         | xxx  | xx                 | xxx     | xx     |

65 As indicated, the polymeric modifier increased the affinity of the polyolefinic composition for dyes in general.

#### Example 2

70 In accordance with Example 1, the predried and ground copolymeric modifier was mixed with the polyolefin, processed and evaluated. For comparison purposes, a similarly prepared polyvinyl pyrrolidone homopolymer (2d) was also evaluated after similar processing. The results 75 of the evaluation are tabulated below:

TABLE

| Sample | Percent Add | Dispersibility in Polyolefin | Percent of A <sup>1</sup> | Dyestuff Class |      |                   |         |        |
|--------|-------------|------------------------------|---------------------------|----------------|------|-------------------|---------|--------|
|        |             |                              |                           | Disperse       | Acid | Prometalized Acid | Mordant | Direct |
| 2a     | 2           | Excellent                    | 1.6                       | xx             | x    | x                 |         |        |
| 2b     | 5           | Good                         | 4                         | xxx            | xx   | xx                | x       |        |
| 2c     | 10          | do                           | 8                         | xxx            | xxx  | xx                | x       |        |
| 2d     | 5           | Poor                         | 5                         | xx             | x    | xxx               | xxx     | 0      |

<sup>1</sup> N-vinyl pyrrolidone.

As is apparent from the table above, the homopolymer (polyvinyl pyrrolidone) was not uniformly dispersed and did not dye as well as the copolymer (80% N-vinyl pyrrolidone/20% dimethylaminoethyl methacrylate). 20

*Example 3*

In accordance with the procedure of Example 1, similar tests were made and the results were set forth in the table which follows: In this case, the modifiers utilized were the copolymers heretofore listed in Markush form in column 3 and the following homopolymers, *viz.*:

- 2A, 3A, 4A—polyvinyl pyrrolidone  
 5A, 6A—polyisoprenyl pyrrolidone  
 7A—polyacrylyl pyrrolidone  
 8A—polyvinyl methylpyrrolidone  
 9A—polyvinyl morpholine  
 10A, 11A—polyvinyl morpholinone  
 12A, 13A—polyvinyl caprolactam

- 14A—polyvinyl oxazolidinone  
 15A—polyvinyl morpholinone  
 16A—polyvinyl benzamidoazole  
 17A—polyvinyl phthalamide  
 18A—polyvinyl diglycolimide  
 19A—polyvinyl oxazolidone

As is apparent from the table below, the copolymeric modifier in all cases increased the affinity of the composition for dyes over and above the level achieved when the modifier utilized represented a corresponding homopolymer. 25

*Example 4*

In accordance with the procedure of Example 1, fiber samples were prepared and tested at the 5% level with the following modifiers, *viz.* (4a) a copolymer of 90% N-vinyl pyrrolidone with 10% 2-vinylpyridine, (4b) a 2-vinylpyridine homopolymer, (4c) a polyethylene imine and (4d) a polydimethylaminoethyl methacrylate. The

TABLE

| Modifier | Percent ratio (if any) | Percent add | Percent A <sup>1</sup> | Dispersibility in Polyolefin | Dyeability with |                         |
|----------|------------------------|-------------|------------------------|------------------------------|-----------------|-------------------------|
|          |                        |             |                        |                              | Acid dyes       | Pre-metalized acid dyes |
| 2        | 95/5                   | 7           | 6.7                    | Fair                         | xxx             | xxx                     |
| 2a       |                        | 7           | 7                      | Poor                         | x               | x                       |
| 3        | 85/15                  | 3           | 2.6                    | Gd/ex                        | xx              | xx                      |
| 3a       |                        | 3           | 3                      | Poor/fair                    | 0               | 0                       |
| 4        | 80/20                  | 5           | 4                      | Good                         | xx              | xx                      |
| 4a       |                        | 4           | 4                      | Poor/fair                    | 0               | x                       |
| 5        | 80/20                  | 5           | 4                      | Good                         | xx              | xxx                     |
| 5a       |                        | 4           | 4                      | Poor/fair                    | 0               | x                       |
| 6        | 70/30                  | 3           | 2.1                    | Excellent                    | xx              | xx                      |
| 6a       |                        | 2           | 2                      | Poor/fair                    | 0               | 0                       |
| 7        | 90/10                  | 10          | 9                      | Fair/good                    | xxx             | xxx                     |
| 7a       |                        | 9           | 9                      | Very poor                    | x               | x                       |
| 8        | 90/10                  | 10          | 9                      | Good                         | xxx             | xxx                     |
| 8a       |                        | 9           | 9                      | Very poor                    | x               | x                       |
| 9        | 70/30                  | 5           | 3.5                    | Very poor                    | xx              | xx                      |
| 9a       |                        | 3.5         | 3.5                    | Good/excel                   | xxx             | xx                      |
| 10       | 70/30                  | 7           | 4.9                    | Poor/fair                    | 0               | x                       |
| 10a      |                        | 5           | 5                      | Good                         | xxx             | xxx                     |
| 11       | 70/30                  | 5           | 3.5                    | Poor                         | 0               | x                       |
| 11a      |                        | 3.5         | 3.5                    | Good/excel                   | xx              | xx                      |
| 12       | 80/20                  | 7           | 5.6                    | Poor/fair                    | 0               | 0                       |
| 12a      |                        | 6           | 6                      | Poor                         | xx              | xxx                     |
| 13       | 80/20                  | 10          | 8                      | Good                         | xxx             | xxx                     |
| 13a      |                        | 8           | 8                      | Very poor                    | x               | x                       |
| 14       | 95/5                   | 15          | 14                     | Fair/good                    | xx              | xxx                     |
| 14a      |                        | 15          | 15                     | Very poor                    | x               | x                       |
| 15       | 90/10                  | 10          | 9                      | Good                         | xxx             | xxx                     |
| 15a      |                        | 9           | 9                      | Very poor                    | x               | x                       |
| 16       | 70/30                  | 5           | 3.5                    | Good/excel                   | xx              | xxx                     |
| 16a      |                        | 3.5         | 3.5                    | Poor/fair                    | 0               | x                       |
| 17       | 70/30                  | 5           | 3.5                    | Good/excel                   | xxx             | xx                      |
| 17a      |                        | 3.5         | 3.5                    | Poor/fair                    | x               | 0                       |
| 18       | 90/10                  | 10          | 9                      | Fair/good                    | xxx             | xxx                     |
| 18a      |                        | 9           | 9                      | Very poor                    | x               | x                       |
| 19       | 70/30                  | 7           | 4.9                    | Good                         | xxx             | xxx                     |
| 19a      |                        | 5           | 5                      | Poor                         | x               | x                       |

<sup>1</sup> Oxygen containing N-heterocyclic monomeric units.

amples were dyed accordingly and the ratings are listed in the table which follows:

| Modifier | Dyestuff Class |      |                     |         |        |
|----------|----------------|------|---------------------|---------|--------|
|          | Disperse       | Acid | Pre-metallized Acid | Mordant | Direct |
| 1        | XXX            | XX   | XX                  | XX      | X      |
| 2        | X              | 0    | 0                   | 0       | 0      |
| 3        | XX             | X    | X                   | 0       | 0      |
| 4        | X              | X    | 0                   | 0       | 0      |

NOTE: The more basic polyvinylpyridine, polyethylene imine, and olydimethylaminoethyl methacrylate, gave poor to fair dyeability because of greater solubility in the polyolefin and a tendency to surface dye blockage. My more hydrophilic, less basic modifiers are less soluble in the polyolefin, and concentrate in the amorphous regions where they form an efficient network for uniform and efficient dyeing with negligible surface dye blockage. Also, while the imine material exhibited some level of dyeability, surface dye blockage with acid and premetallized acid dyes was very severe. Further, the color of the fiber was very dull and the dye rubbed off. In addition, most of the surface dye was removed by dry cleaning with perchloroethylene. The copolymeric modifier of this invention had none of these deficiencies.

Many alternate methods of combining my modifiers with polyolefins are readily available. They may be combined during formation of the polymeric modifier or during actual polymerization of the polyolefin, with or without melting. They may be added to freshly polymerized polyolefin, which is still in solution in a suitable solvent, in the powdered form, or as a solution in a compatible solvent, or merely as a dispersion. They may be added to the polyolefin during precipitation, washing, neutralizing or compounding of the freshly prepared polyolefin prior to drying. This may be accomplished by adding the modifier as a powder or as a solution which is a non-solvent for the polyolefin.

The modifiers may also be melt mixed during processing or blending of the polymer prior to use in extrusion of fiber, film, coating or plastic. It may also be added as a liquid or powder to finely ground or micronized polyolefin polymers and then melt dispersed in situ during hot dip or spray coating or during spreading and heat coating operation. They may be incorporated in polyolefin solutions or emulsion and then applied to surfaces with or without heating.

The level of addition of the modifiers heretofore listed should be between 2 and 20% of the weight of the overall composition. If less than 2% is utilized, significant improvement will not be achieved in dyeability. If an amount greater than 20% is added to the polyolefin, many of the physical properties of the final product, such as fiber or film, are adversely affected. These include loss of strength and a lower resistance to repeated flexing.

The copolymer should contain between 70% and 99% by weight of an oxygen containing N-heterocyclic monomeric unit at which level improved dyeability may be achieved without post treatments and surface blockage. If the copolymer contains between 1% to 30% of a basic monomeric unit, this will contribute towards improved affinity for acid dyes.

However, if the basic monomeric unit is present in an amount greater than 30% by weight, there will be excessive problems in processing. For instance, the modifier will be highly soluble in the polyolefin and less effective in concentration in the amorphous region where needed for improved dyeability. This will be accompanied by excessive surface blockage. Also, if the monomeric unit of a basic nature is present in less than 1% by weight of the copolymer, there will be no appreciable benefit achieved in dyeability.

Prior efforts to develop polymeric modifiers for high melting polyolefins have stressed development and use of specific polymers with relatively high solubility in the polyolefin. These modifiers included polyimines and polyvinylpyridines.

Polyimines have high molecular mobility which ap-

parently gives them some ease of solution in polyolefins. However, this is also a high tendency to sweat out and separate when the combination is made into fiber or film. This material also gives high surface blockage and excessive cracking. On the other hand, soluble polyvinylpyridines confer little or no dyeability on the polyolefin when dissolved therein. This appears to be the case until the preformed modified polyolefin is post treated with epoxy compounds, concentrated acids, alkylating agents, nitrous oxide gas, and alkylene oxides. However, such post treatments are difficult, costly and generally impractical.

Under present concept, I prefer hydrophilic polymeric modifiers which may be soluble in either water or an oxygenated solvent but which are not soluble in the polyolefin. I do prefer modifiers which are fusible and can be dispersed in the polyolefin.

Prior experience with comparatively less hydrophobic fiber forming polymers, such as polyacrylonitrile polymers and polyamides, have shown that the use of hydrophilic, water soluble or dispersible modifiers is impractical, mainly, because excessive amount of the modifier are leached out in scouring and dyeing processes. Surprisingly, I have found that my hydrophilic polymeric modifiers, when melt dispersed in the more hydrophobic polyolefin, have good dispersion stability and are not susceptible to leachage.

I have found that at comparatively low levels of addition, my modifiers confer good dyeability on the polyolefin without the necessity for costly and sometimes impractical post treatments.

My hydrophilic modifiers must be fusible with the polyolefin. This is necessary for the formation of a continuous network of modifiers throughout the polyolefin in order to permit dye penetration and efficient coordination of the dye and modifier throughout the film or fiber.

The use of a non-fusible cross-linked modifier, which results in poor dispersion, is ineffectual. The required modifier network in such a case cannot be formed and the discrete separate particles are surrounded by unmodified areas within the polyolefin matrix. As a result, dyeing is limited to the fiber surface and the dye cannot penetrate into the interior of the fiber where it is most desired.

It is generally recognized that dyeing takes place almost entirely in the more open and readily accessible amorphous areas. When a soluble modifier is utilized, it is usually spread throughout the amorphous and crystalline areas of the polyolefin. As a result, the modifier in the crystalline areas is not available for improvement in dyeability. It also interferes with crystallization and adversely affects strength and thermal stability. However, my non-soluble, hydrophilic, polymeric modifiers are not sufficiently compatible to be a part of the more uniform and denser crystalline areas. It appears to concentrate in the more amorphous areas where it is necessary for dyeability. It has also been found that an increase in molecular weight of my modifiers, further reduces compatibility with stereoregular polyolefins and promotes concentration of the modifier in the more amorphous regions where it may improve the dyeability of the polyolefinic matrix.

Obviously, many modifications and variations of the present invention are possible in the light of the above teaching. For instance, the modifiers of this invention may be used to increase opacity and the affinity of the polyolefin for finishes. They may also be used to improve the printable of the polyolefin, increase the adhesion of the polyolefin to other materials, or to reduce the overall static propensity of the final product. It is therefore to be understood that within the scope of the appended claims, the invention may be practiced otherwise than as specifically described.

I claim:

1. A polymeric composition having improved affinity for dyes comprising a matrix of stereoregular polyolefin taken from the group consisting of polypropylene,

polymethylpentene, and polymethylbutene;

said matrix having dispersed therein between 2% and 20% of a copolymer selected from the group consisting of:

- (a) 80% N-vinyl pyrrolidone/20% dimethylaminoethyl methacrylate,
- (b) 80% N-vinyl pyrrolidone/20% methyl ethylene imine,
- (c) 70% N-isopropenyl pyrrolidone/30% dimethylaminoethyl acrylamide,
- (d) 90% N-acrylyl pyrrolidone/10% N-vinyl pyrrole,
- (e) 70% N-vinyl morpholine/30% N-vinyl carbazole,
- (f) 70% N-vinyl morpholinone/30% N-butyl vinyl quinoline,
- (g) 80% N-vinyl caprolactam/20% N-vinyl succinimide,
- (h) 95% N-vinyl oxazolidinone/5% laurylaminoethyl methacrylate,
- (i) 70% N-vinyl methylpyrrolidone/30% butylaminoethyl methacrylate, and
- (j) 90% N-vinyl pyrrolidone/10% 2-vinyl pyridine, all said percentages being by weight.

2. The combination of claim 1 wherein said copolymer is 80% by weight N-vinyl pyrrolidone in combination with 20% dimethylaminoethyl methacrylate.

3. The combination of claim 1 wherein said copolymer is 95% by weight N-vinyl oxazolidinone in combination with 5% by weight laurylaminoethyl methacrylate.

4. The combination of claim 1 wherein said copolymer is 70% by weight N-vinyl morpholine in combination with 30% by weight N-vinyl carbazole.

5. The combination of claim 1 wherein said copolymer is 70% by weight N-vinyl morpholinone in combination with 30% by weight N-butyl vinyl quinoline.

6. The combination of claim 1 wherein said copolymer is 80% by weight N-vinyl caprolactam in combination with 20% by weight N-vinyl succinimide.

#### References Cited by the Examiner

##### UNITED STATES PATENTS

|           |         |                |       |         |
|-----------|---------|----------------|-------|---------|
| 2,527,863 | 10/1950 | Webb           | ----- | 260—895 |
| 2,628,214 | 2/1953  | Pinkney et al. | ----- | 260—897 |
| 2,927,904 | 3/1960  | Cooper         | ----- | 260—889 |
| 3,003,845 | 10/1961 | Ehlers         | ----- | 260—895 |
| 3,022,267 | 2/1962  | Young          | ----- | 260—895 |
| 3,115,478 | 12/1963 | Ginstiniani    | ----- | 260—895 |

##### FOREIGN PATENTS

|           |        |               |
|-----------|--------|---------------|
| 1,228,539 | 3/1960 | France        |
| 834,160   | 5/1960 | Great Britain |
| 850,435   | 5/1960 | Great Britain |

MURRAY TILLMAN, Primary Examiner.

D. J. BREZNER, Assistant Examiner.